

Nov. 7, 1972

SHUI SATO ET AL  
LIGHT-SENSITIVE SILVER HALIDE PHOTOGRAPHIC EMULSION  
FOR MICROFILM USE  
Filed Dec. 9, 1968

3,702,251



1

3,702,251

### LIGHT-SENSITIVE SILVER HALIDE PHOTOGRAPHIC EMULSION FOR MICROFILM USE

Shui Sato, Kaiichiro Sakazume, and Tsuneo Suga, Tokyo, Japan, assignors to Konishiroku Photo Industry Co., Ltd., Tokyo, Japan

Filed Dec. 9, 1968, Ser. No. 782,169  
Int. Cl. G03c 1/14

U.S. Cl. 96—124

6 Claims

### ABSTRACT OF THE DISCLOSURE

Silver halide photographic emulsions for microfilm use are sensitized by incorporating thereinto, two or more dyes of the Formula (I) and one compound of the Formula (II) in combination:



wherein R<sub>1</sub>, R<sub>3</sub>, R<sub>4</sub> and R<sub>6</sub> are independently selected from the group consisting of lower alkyl group, a carboxyalkyl group or a sulfoalkyl group, with the proviso that at least one of R<sub>1</sub>, R<sub>3</sub>, R<sub>4</sub> and R<sub>6</sub> is a carboxyalkyl, sulfoalkyl or sulfalkoxyalkyl group; R<sub>2</sub> is hydrogen atom or a lower alkyl group; R<sub>5</sub> is a lower alkyl group; Y is hydrogen atom, chlorine atom, a lower alkyl group or a lower alkoxy group; Y<sub>2</sub> is hydrogen atom or a lower alkyl group with the proviso that when Y<sub>1</sub> is chlorine, Y<sub>2</sub> is methyl; Z is a group capable of forming, together with the adjacent nitrogen and carbon atoms, a heterocyclic ring; X is an anion; and 1, n and m are each 1 or 2.

This invention relates to sensitized light-sensitive silver halide photographic emulsions for microfilm use. More particularly this invention relates to a light-sensitive silver halide photographic emulsion suited for microfilm, which comprises two or more sensitizing dyes of the general Formula (I) in combination with one sensitizing dye of the general Formula (II):



wherein R<sub>1</sub>, R<sub>3</sub>, R<sub>4</sub> and R<sub>6</sub> are independently selected from the group consisting of a lower alkyl radical, a carboxy-

2

alkyl group, a sulfoalkyl group and a sulfoalkoxyalkyl group; R<sub>2</sub> is hydrogen atom or a lower alkyl group; R<sub>5</sub> is an alkyl group, with the proviso that at least one of R<sub>1</sub>, R<sub>3</sub>, R<sub>4</sub> and R<sub>6</sub> is a carboxyalkyl, sulfoalkyl or sulfoalkoxyalkyl group; Y<sub>1</sub> is hydrogen atom, chlorine atom, an alkyl group or an alkoxy group; Y<sub>2</sub> is hydrogen atom or an alkyl group, with the proviso that Y<sub>2</sub> is methyl when Y<sub>1</sub> is chlorine atom; Z is an atomic grouping capable of forming, together with the adjacent nitrogen and carbon atoms, a heterocyclic ring such as thiazoline, benzothiazole, benzoselenazole, etc.; X is an anion; and r, m and n are each 1 or 2.

For the purpose of long term storage or reproduction of various printed matters including official documents, bonds, drawings, etc., photo-recording using microfilm is widely known. In such case, the color of the original to be photographed varies over the entire range of the visible spectrum. Further, the above-said photo-recording is usually made under a tungsten lamp having many number of absorptions in the long wavelength region. Therefore, the inherent sensitivity of the usual silver halide photographic emulsion is not sufficient if said emulsion is intended to be used in a light-sensitive photographic material for copying art such as microfilm recording. For this purpose, it is necessary to have the usual silver halide photographic emulsion panchromatically sensitized.

It is an object of the present invention to provide a light-sensitive silver halide photographic emulsion having strengthened sensitivity over the entire visible spectrum and particularly at long wavelengths and further having good sharpness and stability.

We have now found that a light-sensitive silver halide photographic emulsion added to two or three members of the compounds of the above-indicated general Formula I in combination with one member of the compounds of the above-indicated general Formula II can show the desired improved sensitivity for microfilm recording application.

Typical compounds of the general Formulas I and II are listed below, without limiting the scope of this invention thereto.

45 Compounds of the general formula (I)

No. (1)



No. (2)



No. (3)



70

No. (4)



No. (5)



No. (6)



No. (7)



No. (8)



No. (9)



No. (10)



## Compounds of the General Formula (II)

No. (11)



No. (12)



No. (13)



40 The joint use of two or three compounds of the general Formula I with a compound of the general Formula II enables one to obtain such particular spectral sensitization of a light-sensitive silver halide emulsion as has never been observed by the sole use of the individual compounds. Thus, the photographic emulsion can be imparted with sufficient spectral sensitivity over the entire visible spectrum, so that the said emulsion is excellent in photographic reproducitvity. Further, this emulsion, when used for a microfilm can show good photographic characteristics. A still further advantage of this invention is that the distribution of sensitivity maxima can be optionally determined by varying the types and proportions of the compounds of the general Formulas I and II. Furthermore, the sensitizing compounds used in this invention do not cause any adverse interaction with other photographic additives which may be present in the emulsion. A microfilm prepared from the emulsion of the invention is entirely free from deterioration of photographic properties (e.g. decrease of spectral sensitivity, etc.) during storage.

60 All the combinations of any two or three of the compounds of the general Formula I with any one of the compounds of the general Formula II are effective for the purpose of the invention. As stated above, however, the particular combination wherein at least one of the sensitizing dyes used has a solubilizing carboxyalkyl or sulfoalkyl substituent is preferred because color staining which is usually observed after development can be remarkably decreased as the result of increased hydrophilic property.

70 Addition of the compounds of the general Formulas I and II to a silver halide photographic emulsion may be made in a conventional manner. For example, these compounds are dissolved into a water-miscible organic solvent such as methanol, ethanol, etc., to give a solution which is then added to a photographic emulsion. Alternatively, a

plurality of solutions are prepared by dissolving the individual compounds into an organic solvent and then added to a photographic emulsion. The incorporation of the sensitizing compounds into a photographic emulsion may be made at any stage during the preparation of said emulsion. Usually it is preferred to make this addition just before the completion of the second ripening. The total amount of the sensitizing compounds used may vary depending on the type of photographic emulsion and the kinds of the sensitizing compounds, but it usually is within the range of 10-200 mg. per kilogram of the photo-

Sodium carbonate (monohydrate) ----- 30.0  
Potassium bromide ----- 5.0  
Water to make up 1.0 l.

5 The results of measurement of photographic speed and color staining are set forth in Table 1. For comparison, the test results of light-sensitive silver halide photographic films sensitized by the sole use of individual sensitizing dyes are also shown in Table 1. The values for color staining is expressed as color density measured by using a filter.

10

TABLE 1

| Compound number | Amount (ml.) <sup>1</sup> | Compound(s) used |                           |                 | Amount (ml.) <sup>1</sup> | Relative speed  |                 |               |      |       | Color stain |
|-----------------|---------------------------|------------------|---------------------------|-----------------|---------------------------|-----------------|-----------------|---------------|------|-------|-------------|
|                 |                           | Compound number  | Amount (ml.) <sup>1</sup> | Compound number |                           | White light (W) | Green light (G) | Red light (R) | G/W  | R/W   |             |
| No. (1) -----   | 100 -----                 |                  |                           |                 |                           | 55 -----        |                 |               |      |       | 0.02        |
| No. (6) -----   | 100 -----                 |                  |                           |                 |                           | 75 -----        | 45              | 25            | 0.60 | 0.33  | 0.02        |
| No. (13) -----  | 100 -----                 |                  |                           |                 |                           | 65 -----        | 35              | -----         | 0.54 | ----- | 0.03        |
| No. (1) -----   | 30                        | No. (6) -----    | 50                        | No. (13) -----  | 30                        | 105 -----       | 75              | 50            | 0.72 | 0.48  | 0.02        |
| Do -----        | 50                        | do -----         | 100                       | do -----        | 30                        | 110 -----       | 85              | 60            | 0.77 | 0.55  | 0.02        |
| No. (2) -----   | 100 -----                 |                  |                           |                 |                           | 40 -----        |                 |               |      |       | 0.02        |
| No. (5) -----   | 100 -----                 |                  |                           |                 |                           | 85 -----        | 55              | 35            | 0.65 | 0.41  | 0.03        |
| No. (12) -----  | 100 -----                 |                  |                           |                 |                           | 75 -----        | 40              | -----         | 0.53 | ----- | 0.03        |
| No. (2) -----   | 30                        | No. (6) -----    | 50                        | No. (12) -----  | 30                        | 100 -----       | 75              | 50            | 0.75 | 0.60  | 0.02        |
| Do -----        | 50                        | do -----         | 100                       | do -----        | 30                        | 105 -----       | 75              | 60            | 0.71 | 0.57  | 0.02        |

<sup>1</sup> 0.1% MeOH solution added to 1 kg. emulsion.

graphic emulsion. Any types of light-sensitive silver halide emulsions can be sensitized according to the present invention and typically include silver chloride, silver bromide, silver iodobromide, silver chlorobromide and silver chloroiodide emulsions. The light-sensitive silver halide photographic emulsion sensitized according to this invention may contain gold sensitizer, sulfur sensitizer, reductive sensitizer or polyalkyleneoxide sensitizer, and further may contain any known photographic additives such as stabilizer, coating aid, hardener, etc.

The present invention will now be explained in detail in connection with the following examples without limiting the scope of the invention thereto.

#### EXAMPLE 1

A silver chlorobromide solution for copying use is prepared, which contains 50 mol. percent of this emulsion, just before the completion of the second ripening, the indicated amount of various compounds set forth in Table 1 is added in the form of an 0.1% methanol solution at a high temperature. Then, the emulsion is coated on a film base and dried.

The light-sensitive silver halide photographic film (microfilm) thus obtained has good spectral sensitivity over the entire visible spectrum and is particularly excellent in spectral sensitivity at long wavelengths. This photographic film does not suffer from any interaction due to the coexistence of the sensitizers and photographic additives and is entirely free from color staining after development. When this film is used in copying, it is possible to obtain good reproduction from an original having spectral absorptions over the entire visible spectrum even by using a tungsten lamp as light source.

The photographic film is exposed to light according to the JIS method K-7609 and then treated at 20° C. for 4 minutes with a developer of the following formulation:

|                                    |      |    |
|------------------------------------|------|----|
| Metol -----                        | 1.0  | G. |
| Sodium bisulfite (anhydrous) ----- | 75.0 |    |
| Hydroquinone -----                 | 9.0  |    |

35 As is apparent from the above table, the microfilms of the present invention are highly improved in photographic speed to white light in comparison with those prepared by the sole use of the individual compounds of the general Formula I and II. Further, the films of this 40 invention have an increased ratio of both G/W and R/W. Good spectral sensitivity over the entire visible spectrum is obtained.

#### EXAMPLE 2

45 The same silver chlorobromide emulsion as used in Example 1 is subjected to a second ripening with a gold sensitizer to obtain maximum sensitivity. Just before the completion of said second ripening, each one kilogram portion of the emulsion is added at a high temperature 50 with the indicated amount of varying compound in the form of an 0.1% methanolic solution, as shown in Table 2. After the completion of the second ripening, the emulsion is added with an optimum amount of 4-hydroxy-6-methyl-1,3,3a,7-tetrazaindene. The thus obtained emulsion is coated on a film base and then dried.

55 The light-sensitive silver halide photographic film (microfilm) has good spectral sensitivity over the entire visible spectrum and is particularly excellent in spectral sensitivity at long wavelengths. This photographic film does not suffer from any adverse effect due to the coexistence of the sensitizers and photographic additives and is entirely free from color staining after development. Further, there is not observed any deterioration of photographic properties even after the storage of the film for a 60 long period of time. When this film is used in copying, it is possible to obtain good reproduction from an original having spectral absorptions over the entire visible spectrum even by using a tungsten lamp as light source.

The photographic film is exposed to light according to 65 the JIS method K-7609 and then treated with a developer in the same manner as in Example 1. Photographic speed and fog are set forth in Table 2. For comparison, the test results of light-sensitive silver halide photographic films sensitized by the sole use of individual sensitizing dyes are also shown.

TABLE 2

| Compound number | Compound(s) used |                           | Amount (ml.) <sup>1</sup> | Compound number | Amount (ml.) <sup>1</sup> | Compound number | Amount (ml.) <sup>1</sup> | Compound number | Fresh |             | Incubated at 65° C. for 3 days |           | Incubated at 65° C. for 3 days at 80% R.H. |             | Sensitivity maximum m $\mu$ |
|-----------------|------------------|---------------------------|---------------------------|-----------------|---------------------------|-----------------|---------------------------|-----------------|-------|-------------|--------------------------------|-----------|--------------------------------------------|-------------|-----------------------------|
|                 | Compound number  | Amount (ml.) <sup>1</sup> |                           |                 |                           |                 |                           |                 | Fog   | White light | Green light                    | Red light | Fog                                        | White light |                             |
| No. (1)         | 100              | ...                       | 0.02                      | 56              | 30                        | 0.02            | 55                        | 30              | 0.03  | 55          | 30                             | 60        | 60                                         | 36          | 430                         |
| No. (4)         | 100              | ...                       | 0.02                      | 80              | 35                        | 0.02            | 85                        | 35              | 0.02  | 80          | 35                             | 66        | 66                                         | 36          | 620                         |
| No. (10)        | 100              | ...                       | 0.02                      | 80              | 35                        | 0.04            | 65                        | 35              | 0.03  | 65          | 35                             | 70        | 40                                         | ...         | 540                         |
| No. (11)        | 100              | ...                       | 0.02                      | 65              | 40                        | 0.03            | 70                        | 35              | 0.02  | 70          | 35                             | 90        | 90                                         | 55          | 600                         |
| No. (12)        | 100              | ...                       | 0.02                      | 70              | 40                        | 0.02            | 110                       | 85              | 0.02  | 105         | 95                             | 120       | 110                                        | 95          | 65                          |
| No. (1)         | 30               | No. (12)                  | 60                        | No. (12)        | 30                        | 0.02            | 106                       | 90              | 0.02  | 105         | 95                             | 120       | 110                                        | 105         | 60                          |
| No. (1)         | 30               | No. (10)                  | 60                        | No. (10)        | 30                        | 0.02            | 120                       | 95              | 0.02  | 120         | 95                             | 120       | 110                                        | 105         | 620                         |
| No. (1)         | 50               | do                        | 40                        | No. (10)        | 20                        | 0.02            | 105                       | 80              | 0.02  | 105         | 80                             | 115       | 105                                        | 85          | 70                          |
| No. (1)         | 50               | do                        | 40                        | No. (10)        | 30                        | 0.02            | 115                       | 85              | 0.02  | 115         | 85                             | 115       | 105                                        | 85          | 70                          |
| No. (1)         | 50               | do                        | 50                        | No. (10)        | 30                        | 0.02            | 115                       | 85              | 0.02  | 115         | 85                             | 115       | 105                                        | 85          | 70                          |

<sup>1</sup> 0.1% MeOH solution added to 1 kg. emulsion.

As is apparent from the above table, the light-sensitive silver halide photographic films of the present invention are highly improved in spectral sensitivity in comparison with those prepared by the sole use of the individual compounds of the general Formulae I and II. Further these films have good spectral sensitivity over the entire visible spectrum. Stability of the films is satisfactory to make them free from fogging, decrease in photographic speed, etc., over a long period of time.

In the attached drawings, FIG. 1 is a spectral sensitivity curve of the silver chlorobromide emulsion used as the starting material of this example; FIG. 2 (I), (II) and (III) are spectral sensitivity curves of the said emulsion when added with each of the compounds No. (1), No. (4) and No. (12) respectively; and FIG. 3 is a spectral sensitivity curve of the said emulsion when added with the combination of the compounds No. (1), (4) and (12) according to the present invention. As is clear from the drawing, the light-sensitive silver halide photographic emulsion of the invention is highly improved in spectral sensitivity over the entire visible spectrum in comparison with a photographic emulsion sensitized with a single compound of the general Formulas I and II.

What is claimed is:

1. A light-sensitive silver halide photographic emulsion for microfilm, which comprises in combination two or three sensitizing dyes of the compounds of the general Formula I:



and one sensitizing dye of the compounds of the general Formula II:



wherein R<sub>1</sub>, R<sub>3</sub>, R<sub>4</sub> and R<sub>6</sub> are independently selected from the group consisting of a lower alkyl group, a carboxy-alkyl group or a sulfoalkyl group, with the proviso that at least one of R<sub>1</sub>, R<sub>3</sub>, R<sub>4</sub> and R<sub>6</sub> is a carboxyalkyl, sulfoalkyl or sulfalkoxyalkyl group; R<sub>2</sub> is hydrogen atom or a lower alkyl group; R<sub>5</sub> is a lower alkyl group; y is hydrogen atom, chlorine atom, a lower alkyl group or a lower alkoxy group; Y<sub>2</sub> is hydrogen atom or a lower alkyl group with the proviso that when Y<sub>1</sub> is chlorine, Y<sub>2</sub> is methyl; Z is a group capable of forming, together with the adjacent nitrogen and carbon atoms, a heterocyclic ring; X is an anion; and r, n and m are each 1 or 2.

2. A light-sensitive silver halide photographic emulsion for microfilm use, as claimed in claim 1, wherein said combination consists of 3,3'-diethyl-thiazolino-carbocyanine iodide, 3,3' - sulfoethoxyethyl - 9 - methyl-thiacarbocyanine triethylamine and (3 - carboxyethyl - 5 - methoxybenzoxazolo) - 1,3 - diethyl - 5,6 - dichloro-benzimidazolo-carbocyanine bromide.

3. A light-sensitive silver halide photographic emulsion for microfilm use, as claimed in claim 1, wherein said combination consists of 3,3' - dicarboxyethyl-thiazolino-carbocyanine bromide, 3,3' - hydroxyethyl - 9 - methyl-thiacarbocyanine iodide and (3 - ethyl - 5 - chloro - 6 - methyl-benzoxazolo) - (1 - ethyl - 3 - sulfobutyl - 5,6 - dichloro-benzimidazolo)-carbocyanine.

4. A light-sensitive silver halide photographic emulsion for microfilm use, as claimed in claim 1, wherein said

combination consists of 3,3' - diethyl-thiazolino-carbo-cyanine iodide, 3,3' - disulfobutyl - 9 - methyl-thia-carbo-cyanine iodide and (3 - ethyl - 5 - chloro - 6-methyl-benzoxazolo) - (1 - ethyl - 3 - sulfobutyl - 5,6-dichloro-benzimidazolo)-carbocyanine.

5. A light-sensitive silver halide photographic emulsion for microfilm use, as claimed in claim 1, wherein said combination consists of 3,3' - diethyl-thiazolino-carbo-cyanine iodide, 3,3' - disulfobutyl - 9 - methyl-thia-carbo-cyanine iodide, 3,3'-disulfobutyl-9-methyl-benzselenazolo-carbocyanine and (3-ethyl-benzoxazolo)-(1-ethyl-3-ethyl-5,6-dichloro-benzimidazolo)-carbocyanine iodide.

6. A microfilm which comprises a film base and, supported thereon, a layer of the smulsion as claimed in claim 1.

## References Cited

## UNITED STATES PATENTS

|             |        |               |       |        |
|-------------|--------|---------------|-------|--------|
| 3,173,791   | 3/1965 | Kalenda       | ----- | 96—104 |
| 3,431,110   | 3/1969 | Ficken et al. | ----- | 96—104 |
| 5 3,463,640 | 8/1969 | Ficken et al. | ----- | 96—104 |

## FOREIGN PATENTS

|           |        |        |       |     |
|-----------|--------|--------|-------|-----|
| 1,137,701 | 6/1957 | France | ----- | 1—7 |
|-----------|--------|--------|-------|-----|

10 WILLIAM D. MARTIN, Primary Examiner

B. D. PIANALIO, Assistant Examiner

U.S. Cl. X.R.

15 96—137